# EUROPEAN PATENT SPECIFICATION

(11) **EP 1 567 692 B1**
(45) Date of publication and mention of the grant of the patent: **21.11.2007**
(21) Application number: 03775701.0
(22) Date of filing: 03.12.2003
(51) Int. Cl.: C25C 3/12

(54) **A METHOD OF CONDITIONING IRON ALLOY-BASED ANODES FOR ALUMINIUM ELECTROWINNING CELLS**
VERFAHREN ZUR AKTIVIERUNG VON ANODEN AUF BASIS VON EISEN-LEGIERUNGEN FÜR ALUMINIUM-ELEKTROGEWINNUNGSZELLEN
PROCEDE DE CONDITIONNEMENT D'ANODES A BASE D'ALLIAGE DE FER POUR DES CELLULES D'EXTRACTION ELECTROLYTIQUE D'ALUMINIUM

(30) Priority: 03.12.2002 WO PCT/IB02/05112
(43) Date of publication of application: 31.08.2005
(73) Proprietor: MOLTECH Invent S.A., 1520 Luxembourg (LU)
(72) Inventor: DURUZ, Jean-Jacques, CH-1204 GENEVA (CH); DE NORA, Vittorio, none NASSAU (BS)
(74) Representative: Cronin, Brian Harold John
(86) International application number: PCT/IB2003/005713
(87) International publication number: WO 2004/050956

(56) References cited:
- WO-A-01/42536
- WO-A-03/014420
- US-A- 5 904 828

## Description

### Field of the Invention

This invention relates to the conditioning of iron alloy based aluminium electrowinning anodes to form an integral electrochemically active iron-based oxide layer thereon, anodes so conditioned, aluminium electrowinning cells with such anodes and the production of aluminium in such cells.

### Background Art

The technology for the production of aluminium by the electrolysis of alumina, dissolved in molten cryolite containing salts, at temperatures around 950°C is more than one hundred years old. This process and the cell design have not undergone any great change or improvement and carbonaceous materials are still used as electrodes and cell linings.

Using metal anodes in aluminium electrowinning cells would drastically improve the aluminium process by reducing pollution and the cost of aluminium production. Many patents have been filed on non-carbon anodes but none has found commercial acceptance, also because of economical reasons.

US Patents 4,614,569 (Duruz/Derivaz/Debely/Adorian), 4,680,094 (Duruz), 4,683,037 (Duruz) and 4,966,674 (Bannochie/Sherriff) describe non-carbon anodes for aluminium electrowinning coated with a protective coating of cerium oxyfluoride, formed in-situ in the cell or pre-applied, this coating being maintained by the addition of a cerium compound to the molten cryolite electrolyte. EP Patent application 0 306 100 (Nyguen/Lazouni/Doan), US Patents 5,069,771, 4,960,494 and 4,956,068 (all Nyguen/Lazouni/Doan) describe metallic anode substrates which may be further covered with such an in-situ formed protective cerium oxyfluoride layer.

US Patent 5,510,008 (Sekhar/Liu/Duruz) discloses an anode made from an inhomogeneous porous metallic body obtained by micropyretically reacting a powder mixture of nickel, iron, aluminium and possibly copper and other elements. An electrochemically active oxide-based outer portion is formed by in-situ polarisation.

WO00/06803 (Duruz/de Nora/Crottaz), WO00/06804 (Crottaz/Duruz) and WO01/42534 (de Nora/Duruz) disclose anodes produced from nickel-iron alloys which are surface oxidised to form a coherent and adherent outer iron oxide-based layer whose surface is electrochemically active surface.

WO01/42534 (Duruz/Nguyen/de Nora) discloses a nickel-iron alloy aluminium electrowinning anode with an openly porous electrochemically active surface produced by removal of iron from the surface, in particular by electrolytic dissolution of iron.

WO00/06805 (de Nora/Duruz) discloses an aluminium electrowinning anode having a metallic anode body which can be made of various alloys, for example a nickel-iron-copper alloy. The surface of the anode body is oxidised by anodically evolved oxygen to form an integral electrochemically active oxide-based surface layer. The oxidation rate of the anode body is equal to the rate of dissolution of the surface layer into the electrolyte. This oxidation rate is controlled by the thickness and permeability of the surface layer which limits the diffusion of anodically evolved oxygen to the anode body.

WO01/42536 (Duruz/Nguyen/de Nora) discloses an aluminium electrowinning anode made form a nickel-iron alloy having an openly porous outer portion which consists predominantly of nickel metal and which is obtainable by removal of iron from the alloy.

WO01/42534 (de Nora/Duruz), WO02/070785 (Nguyen/de Nora), WO02/083990 (de Nora/Nguyen), WO02/083991 (Nguyen /de Nora), WO03/014420 (Nguyen/Duruz/de Nora), WO03/078695 (Nguyen/de Nora) and WO03/087435 (Nguyen/de Nora) disclose further metal-based aluminium electrowinning anodes.

Metal or metal-based anodes are highly desirable in aluminium electrowinning cells instead of carbon-based anodes. Usually, the anodes are pre-oxidised in an oxidising atmosphere before use to produce an electrochemically active oxide layer thereon. In practice, prior to insertion into the cell, the metal-based anodes are usually pre-heated above the molten electrolyte to inhibit thermal shocks in the electrolyte and its solidification when the anode is immersed.

### Objects of the Invention

A major object of the invention is to provide a method of conditioning an iron-based alloy anode for aluminium electrowinning to increase its lifetime and improve its electrical conductivity during use.

Another object of the invention is to provide a method of conditioning an iron-based alloy anode to form an active anode surface that has a high electrochemical activity for the oxidation of oxygen ions for the formation of bimolecular gaseous oxygen and a low solubility in the electrolyte.

A further object of the invention is to provide a method of conditioning an iron-based alloy anode to form an integral electrochemically active oxide layer with an improved density and coherence and with limited ionic conductivity for oxygen ions and a low electrical resistance.

Yet another object of the invention is to provide a method of conditioning an aluminium electrowinning anode which is made of readily available alloys(s).

Yet a further object of the invention is to provide an aluminium electrowinning anode which is made of readily available alloys(s) and an aluminium electrowinning cell having such an anode.

### Summary of the Invention

The invention is based on the observation that an integral oxide layer formed by oxidation of an iron-based alloy, in particular an iron-based alloy comprising nickel and/or cobalt, is significantly denser and more coherent when the oxidation of the iron-based alloy is carried out by polarisation thereof in a molten electrolyte under specific conditions compared to oxide layers produced by conventional oxidation in air or by polarisation in a molten electrolyte as disclosed in the prior art.

To produce such a denser and more coherent oxide layer, the anode's active surface is up to immersion into the electrolyte essentially metallic and substantially unreacted with reactive species that form ceramic compounds with metals from the iron-based alloy. Such reactive species include oxygen at or above ambient temperature or fluorine-containing gases that could contact the anode while pre-heating the anode above the cell.

It has been found that the formation of such ceramic compounds on the iron-based alloy before polarisation in the electrolyte impairs the coherence and density of the oxide layer subsequently formed in-situ, which reduces its capacity to limit diffusion of oxygen and leads to thicker oxide layers with greater electrical resistance. It has been observed that this effect is most detrimental when the iron-based alloy is pre-oxidised before electrolysis and also when the iron-based alloy is pre-heated above the electrolyte in the fluorine-containing fumes prior to immersion into the electrolyte.

The invention relates to a method of conditioning a metallic anode structure for producing aluminium in a molten electrolyte containing dissolved alumina. The metallic anode structure has initially an iron-based alloy outer part with an active anode surface which is essentially metallic and free of any ceramic compounds, in particular oxides and fluorides, of metals from the metallic anode structure.

According to the invention, the method comprises the ordered steps of: (a) substantially preventing the essentially metallic active surface free of said ceramic compound from reacting with any reactable species, in particular oxygen and fluorine species, until immersion into a molten electrolyte containing oxygen ions; (b) immersing into the molten electrolyte the metallic anode structure with its essentially metallic active surface free of said ceramic compounds; and (c) polarising the immersed metallic anode structure at a potential above the potential of oxidation of oxygen thereby evolving oxygen on the active anode surface and oxidising the active anode surface to form on the metallic anode structure a dense and coherent integral iron-based oxide layer which is electrochemically active for the oxidation of oxygen and which inhibits diffusion of oxygen towards the metallic anode structure.

The prevention of the metallic active surface from reacting with any reactable species, in particular oxygen and fluorine species, until immersion into a molten electrolyte can be achieved either by protecting the active surface against reaction, for instance by coating the surface with a temporary protective layer, or by avoiding exposure of the active surface to a reactive environment for an extended period of time during which a significant amount of anode constituents at the active surface can react with the environment.

For instance, exposure of a cast iron-based alloy to air at room temperature for a few days would not lead to significant formation of ceramic (oxide) compounds at its surface. However, when the iron-based alloy is' cast and then left unprotected in the atmosphere for a long period of time before use, for example stored several months on a shelf after casting, the surface of the iron-based alloy can become noticeably altered which has been found to reduce the anode's performances, in particular the stability, lifetime and energy efficiency. Moreover, it has been discovered that even a short exposure, e.g. a few minutes, to fluorine-containing gases while pre-heating the anode above a fluoride-based molten electrolyte has a significant deleterious effect.

As opposed to the prior art anode conditioning methods in which the iron-based alloy anodes after casting were kept unprotected until immersion into the molten electrolyte and also preferably were pre-oxidised in a high temperature oxidising atmosphere and/or pre-heated unprotected in fluorine-containing fumes above the molten electrolyte before immersion into the molten electrolyte, the method of conditioning the iron-based alloy anodes of the present invention prevents substantially any reactive interactions between the anode and the environment before immersion into the molten electrolyte.

In case, before use, the anode's alloy contains at its surface a noticeable amount of ceramic compounds produced by reaction of metals from the alloy's surface with a reactive environment, such ceramic compounds should be removed from the alloy's surface before carrying out the method of the invention.

Preferably, the method of the invention includes the step of pre-heating the metallic anode structure, prior to its immersion, to a temperature at which it can be immersed into the molten electrolyte without substantial solidification thereof. During this pre-heating step, the structure's essentially metallic active surface is maintained free of said ceramic compounds by substantially preventing the active anode surface from reacting with the environment during pre-heating before immersion. This is not the case with prior art methods, when the anodes are pre-heated without the inventive conditioning.

Protection of the active anode surface prior to immersion into the molten electrolyte can be achieved by covering the active surface with a temporary protective layer which is substantially impermeable to any species reactable with the active surface and which is removed prior to immersion into the molten electrolyte or dissolves therein as a fugitive coating.

When the anode is pre-heated in a reactive atmosphere prior to immersion, the temporary layer should be heat stable, for instance applied from a ceramic paint, e.g. an alumina-based paint, which is stable also at high temperature. Of course, a heat-stable protective coating can be used even if the anode is not subjected to a preheat treatment.

When the anode structure is not pre-heated in a reactive atmosphere, the temporary layer for longlasting protection at ambient temperature before use, e.g. for storage, can be an organic paint or a substantially impervious wrapping, e.g. made of plastic.

The anode structure can also be pre-heated prior to immersion in an inert atmosphere that is substantially free from any species reactable with the active surface. In this case, no heat stable temporary protective layer is needed during the pre-heating.

The iron-based alloy outer part may comprise one or more elements selected from nickel, cobalt, copper, molybdenum, manganese, titanium, tantalum, tungsten, hafnium, vanadium, zirconium, niobium, chromium, cobalt, aluminium, silicon, carbon and the rare earth metals, in particular yttrium.

In one embodiment, the iron-based alloy outer part, consists essentially of: 45-55 weight% iron; 15-55 weight% in total of nickel and/or cobalt; 0-30 weight% copper; and 0-10 weight% in total of one or more further elements, usually selected from molybdenum, manganese, titanium, tantalum, tungsten, hafnium, vanadium, zirconium, niobium, chromium, cobalt, aluminium, silicon, carbon and the rare earth metals, in particular yttrium.

Further suitable iron-based alloy compositions for the anode structure are disclosed in WO00/40783 (de Nora/Duruz), WO00/06803 (Duruz/de Nora/Crottaz), WO00/06804 (Crottaz/Duruz), WO01/42534 (de Nora/Duruz), WO01/42536 (Duruz/Nguyen/de Nora), WO02/014420 (Nguyen/Duruz/de Nora) and WO03/078695 (Nguyen/de Nora).

The metallic anode structure can be a cast alloy. Casting can be advantageously used to produce anodes of complex shapes, e.g. specially adapted for the circulation of electrolyte. Examples of such anode shapes are disclosed in WO99/02764 (de Nora/Duruz), WO00/40781, WO00/40782 and WO03/006716 (all de Nora).

The metallic anode structure can be quenched and/or annealed prior to immersion into the molten electrolyte, taking care however that the anode's active surface is not exposed to an environment that can substantially react with anode constituents at the active surface.

The invention also relates to a method of conditioning or reconditioning a metallic anode structure for producing aluminium in a molten electrolyte containing dissolved alumina, for example when the metallic anode structure has been impaired by exposure to a reactive environment before use or when the anode structure has been worn during use.

Such a used or impaired metallic anode structure comprises an iron-based alloy outer part having a surface which is covered with ceramic compounds, in particular oxides and fluorides, of metals from the outer part. The conditioning or reconditioning method comprises the steps of: removing substantially all ceramic compounds from the surface of the outer part to form an essentially metallic active anode surface; and then conditioning as described above the metallic anode structure with its essentially metallic active anode surface free of any ceramic compounds.

A further aspect of the invention relates to method of electrowinning aluminium. This method comprises the steps of: conditioning a metallic anode structure as described above including polarising it in a molten electrolyte to form on the anode structure a dense and coherent integral iron-based oxide layer; and electrolysing dissolved alumina in the same or a different molten electrolyte using the conditioned anode structure to evolve oxygen thereon and produce aluminium on a facing cathode.

The dense and coherent integral iron-based oxide layer of the anode structure can be further formed during electrolysis by slow oxidation of the metallic anode structure at the metallic structure/oxide layer interface. Constituents of the dense and coherent integral iron-based oxide layer at the oxide layer/electrolyte interface may slowly dissolve into the electrolyte during electrolysis, preferably at a rate corresponding to the oxidation rate of the metallic anode structure at the metallic structure/oxide layer interface, as disclosed in WO00/06805 (de Nora/Duruz).

As disclosed in WO00/06802 (Duruz/de Nora/Crottaz) the aluminium production molten electrolyte can comprise an amount of dissolved iron species and dissolved alumina sufficient to inhibit significantly dissolution of constituents of the dense and coherent integral iron-based oxide layer at the oxide layer/electrolyte interface.

The anode can be protected against the electrolyte with a cerium oxyfluoride-based outermost coating deposited and/or maintained during use, for example as disclosed in the abovementioned US Patents 4,614,569, 4,680,094, 4,683,037 and 4,966,674.

Preferably, the aluminium production molten electrolyte is maintained at a temperature below 960°C, preferably between 840°C and 940°C.

The aluminium production molten electrolyte can contain NaF and AlF₃ in a molar ratio in the range from 1.2 to 2.4. The alumina content in the aluminium production molten electrolyte is usually below 10 weight%, typically between 5 weight% and 8 weight%.

It is preferred that alumina-depleted electrolyte is circulated away from the electrochemically active iron-based oxide layer, enriched with alumina, and alumina-enriched electrolyte is circulated towards the electrochemically active iron-based oxide layer. Such an electrolyte circulation can be achieved by following the teachings of WO99/41429 (de Nora/Duruz), WO99/41430 (Duruz/Bellò), WO00/40781, WO00/40782, WO01/31088 and WO03/006716 (all de Nora).

Another aspect of the invention relates to an aluminium electrowinning anode structure. This structure comprises an iron-based alloy metallic outer part covered with a dense and coherent integral iron-based oxide layer obtainable by conditioning by the above described method a metallic anode structure having an iron-based alloy outer part with an active anode surface which is essentially metallic and free of any ceramic compounds of metals from the metallic anode structure.

Compared to pre-oxidised anodes or anodes that are pre-heated unprotected in fumes above the molten electrolyte, the anode of the invention exhibits upon use in an aluminium electrowinning cell a more protective denser and more coherent oxide layer which is thinner and more conductive, as demonstrated in the example.

The invention also relates to an aluminium electrowinning anode structure having an iron-based alloy metallic outer part with an active anode surface. Before use, the active surface is essentially metallic and free of any ceramic compounds of metals from the metallic anode structure and is covered with a temporary protection medium. This protective medium substantially prevents ceramic-forming reactions at the essentially metallic anode surface and is separable from the active surface prior to immersion into the molten electrolyte or by contact with the molten electrolyte. Usually, the temporary protection medium is removable prior to immersion into the electrolyte or soluble in the electrolyte.

The temporary protection medium may comprises one or more substantially impervious solid layers. Suitable layers comprise at least one of ceramics, such as alumina, including ceramics applied from colloids, for instance colloidal alumina precursor, such as Nyacol^{™} and/or Condea^{™}, and other colloid precursors of ceramics; metals, in particular reactable metals, such as aluminium, iron, copper, chromium or yttrium, for reacting with possibly diffusing reactive gases; polymers, e.g. plastic, in particular wrapping the anode structure under vacuum or inert gas or carrying one or more of the above layer constituents. Furthermore, the temporary protection medium can comprise an inert liquid or viscous material, such as oil or grease, or an inert gas, such as nitrogen or carbon dioxide, for example within a polymer enclosure or wrapping around the anode structure.

The protective layer can comprise alumina, in particular applied from a paint or slurry, and/or a polymer. The protective layer may also contain metallic particles that trap a possible oxygen diffusion before it reaches the metallic anode surface.

Yet another aspect of the invention relates to an aluminium electrowinning cell comprising at least one oxygen-evolving anode structure as described above.

Preferably, the cell comprises an aluminium-wettable cathode preferably having an aluminium-wettable coating, in particular a drained cathode. Suitable, aluminium-wettable coatings are disclosed in US Patent 5,651,874 (de Nora/Sekhar), and PCT publications WO98/17842 (Sekhar/Duruz/Liu), WO01/42168 (de Nora/Duruz) and WO01/42531 (Nguyen/Duruz/de Nora). Suitable drained cathode designs are disclosed in US Patents 5,683,559, 5,888,360, 6,093,304 (all de Nora), 6,258,246 (Duruz/de Nora), as well as PCT publications WO99/02764 (de Nora/Duruz), WO99/41429 (de Nora/Duruz), WO00/63463 (de Nora), WO01/31086 (de Nora/Duruz) and WO01/31088 (de Nora).

### Detailed Description

The invention will be further described in the following Examples:

### Comparative Example

### Conditioning:

A prior art-type conditioning of an anode was carried out as follows.

An anode was made by pre-oxidising in air at 1100°C for 3 hour a substrate of a cast nickel-iron alloy consisting of 50 weight% nickel, 0.3 weight% manganese, 0.5 weight% aluminium, 0.05 weight% C and 49.15 weight% iron, to form a very thin oxide surface layer on the alloy.

The surface-oxidised anode was cut perpendicularly to the anode operative surface and the resulting section of the anode was subjected to microscopic examination.

The anode before use had an outer portion that comprised an electrolyte-pervious, electrochemically active iron-rich nickel-iron oxide surface layer having a thickness of up to 10-20 micron and, underneath, an iron-depleted nickel-iron alloy having a thickness of about 10-15 µm containing generally round cavities filled with iron-rich nickel-iron oxide inclusions and having a diameter of about 2 to 5 µm. The nickel-iron alloy of the outer portion contained about 75 weight% nickel.

Underneath the outer portion, the nickel-iron alloy had remained substantially unchanged.

### Testing:

An anode prepared as above was pre-heated unprotected in electrolyte fumes above an aluminium electrowinning cell for 20 minutes and then tested therein.

The cell contained a molten electrolyte at 880-890°C consisting essentially of NaF and AlF₃ in a weight ratio NaF/AlF₃ of about 0.7 to 0.8, i.e. an excess of AlF₃ in addition to cryolite of about 24 weight% of the electrolyte, and approximately 5 weight% alumina. The alumina concentration was maintained at a substantially constant level throughout the test by adding alumina at a rate adjusted to compensate the cathodic aluminium reduction. The test was run at a current density of about 0.8 A/cm², and the electrical potential of the anode remained in the range of 4.2 to 4.5 volts throughout the test.

During electrolysis aluminium was cathodically produced while oxygen was anodically evolved which was derived from the dissolved alumina present near the anodes.

After 24 hours, electrolysis was interrupted and the anode was extracted from the cell. The external dimensions of the anode had remained substantially unchanged during the test and the anode showed no signs of damage.

The anode was cut perpendicularly to the anode operative surface and the resulting section of the used anode was subjected to microscopic examination.

It was observed that the anode was covered with an iron oxide surface layer having a thickness of 100 to 120 µm and consisting essentially of Fe₂O₃ with less than 5 weight% nickel oxide.

### Example 1

An anode was made of the same metals as in the comparative Example except that it had an active surface essentially metallic and free of any ceramic compounds, in particular neither oxides nor fluorides, of metals from the anode's surface.

The cold anode was immersed in the molten electrolyte of a cell without prior reaction of the anode's active surface with a reactive environment, i.e. with the active surface essentially metallic and free of said ceramic compounds.

The molten electrolyte was at a temperature of 880-890°C and consisted essentially of NaF and AlF₃ in a weight ratio NaF/AlF₃ of about 0.7 to 0.8, i.e. an excess of AlF₃ in addition to cryolite of about 24 weight% of the electrolyte, and approximately 5 weight% alumina.

Upon immersion of the anode, the electrolyte froze around the anode which prevented electrolysis. After 10 to 15 minutes in the electrolyte, the temperature of the anode had reached the melting point of the electrolyte and the electrolyte contacting the anode had molten thereby permitting electrolysis.

During the test, the alumina concentration was maintained at a substantially constant level throughout the test by adding alumina at a rate adjusted to compensate the cathodic aluminium reduction. The test was run at a current density of about 0.8 A/cm², and the electrical potential of the anode remained in the range of 4.0-4.3 volts throughout the test, i.e. about 0.2 V lower in average than in the above comparative test with a pre-oxidised and fume pre-heated anode.

During electrolysis aluminium was cathodically produced while oxygen was anodically evolved which was derived from the dissolved alumina present near the anodes.

After 24 hours, electrolysis was interrupted and the anode was extracted from the cell. The external dimensions of the anode had remained substantially unchanged during the test and the anode showed no signs of damage.

The anode was cut perpendicularly to the anode operative surface and the resulting section of the used anode was subjected to microscopic examination.

It was observed that the anode was covered with an iron oxide surface layer having a thickness of about 100 µm and consisting essentially of Fe₂O₃ with less than 5 weight% nickel oxide and additionally an outermost layer of oxides of iron and aluminium having a thickness of about 25 µm.

The iron oxide surface layer, with pores of 3 to 5 micron, was denser than the oxide layer of the above comparative anode that had pores of 5 to 10 µm. This greater density of the oxide layer of the anode conditioned according to the invention provides a better protection for the alloy located underneath oxidation and electrolyte attack.

### Example 2

Example 1 was repeated with a pre-heating step of the anode above the molten electrolyte prior to immersion into the electrolyte.

To prevent reaction of the essentially metallic anode surface with electrolyte fumes, the anode was covered with a protective layer of alumina applied from an alumina-based colloidal slurry.

The colloidal slurry comprised an alumina colloid carrier consisting essentially of water and colloidal alumina particles in an amount of 20 weight% of the colloid, for example Nyacol^{™}, and suspended alumina particles in an amount of 60 weight% of the colloidal slurry.

The anode was dipped into the slurry and allowed to dry to produce an alumina coating having a thickness of 0.6 to 1.0 mm covering and protecting the essentially metallic anode surface against reaction with the environment.

After pre-heating the protected anode for about 1 hour in the electrolyte fumes above the molten electrolyte, the anode was immersed with its alumina coating into the molten electrolyte. The protective alumina coating was dissolved almost instantaneously and normal electrolysis could start.

During electrolysis, the anode behaved like the anode in Example 2. After 24 hours, the anode was removed and examined. The anode upon use was not significantly different to the anode of Example 2.

In a variation, the protective effect of the alumina slurry can be improved by substituting half of the suspended alumina particles with suspended metallic particles, such as aluminium, iron and/or copper particles, which trap a possible oxygen diffusion before it reaches the metallic anode surface. Thus, in case the temporary protective coating is not perfectly impervious to the environment, reactive constituents of the environment will react with the metallic particles of the coating and substantially not with the metallic active anode surface.

## Claims

1. A method of conditioning a metallic anode structure for producing aluminium in a molten electrolyte containing dissolved alumina, the metallic anode structure having initially an iron-based alloy outer part with an active anode surface which is essentially metallic and free of any ceramic compounds, in particular oxides and fluorides, of metals from the metallic anode structure, the method comprising the steps of:
a) covering the essentially metallic active surface free of said ceramic compound with a temporary protective layer which is substantially impermeable to any species reactable with the active surface to substantially prevent the active surface from reacting with any reactable species, in particular oxygen and fluorine species, until immersion into a molten electrolyte containing oxygen ions;
b) immersing into the molten electrolyte the metallic anode structure with its essentially metallic active surface free of said ceramic compounds, the temporary protective layer being removed prior to immersion into the molten electrolyte or by contact with the molten electrolyte; and
c) polarising the immersed metallic anode structure to form thereon a dense and coherent integral iron-based oxide layer which is electrochemically active for the oxidation of oxygen and which inhibits diffusion of oxygen towards the metallic anode structure.

2. The method of claim 1, wherein prior to immersion, the metallic anode structure is pre-heated with its essentially metallic active surface maintained free of said ceramic compounds, the protective layer being preferably heat stable.

3. The method of claim 1 or 2, wherein prior to immersion, the metallic anode structure is pre-heated in an atmosphere that is substantially free of any species reactable with the active surface.

4. The method of any preceding claim, wherein the iron-based alloy outer part comprises nickel and/or cobalt.

5. The method of any preceding claim, wherein the iron-based alloy outer part comprises one or more elements selected from copper, molybdenum, manganese, titanium, tantalum, tungsten, hafnium, vanadium, zirconium, niobium, chromium, cobalt, aluminium, silicon, carbon and the rare earth metals, in particular yttrium.

6. The method of claim 4, wherein the iron-based alloy outer part, consists essentially of:
- 45-55 weight% iron;
- 15-55 weight% in total of nickel and/or cobalt;
- 0-30 weight% copper; and
- 0-10 weight% in total of one or more further elements.

7. The method of any preceding claim, wherein the metallic anode structure is a cast alloy, the structure being optionally quenched prior to immersion into the molten electrolyte and/or subjected to an annealing heat treatment prior to immersion into the molten electrolyte.

8. A method of conditioning or reconditioning a metallic anode structure for producing aluminium in a molten electrolyte containing dissolved alumina, the metallic anode structure comprising an iron-based alloy outer part having a surface which is covered with ceramic compounds, in particular oxides and fluorides, of metals from the outer part, said method comprising the steps of:
- removing substantially all ceramic compounds from the surface of the outer part to form an essentially metallic active anode surface; and then
- conditioning according to any preceding claim the metallic anode structure with its essentially metallic active anode surface free of any ceramic compounds.

9. A method of electrowinning aluminium comprising the steps of:
- conditioning according to any preceding claim a metallic anode structure including the step of polarising in a molten electrolyte to form on the anode structure a dense and coherent integral iron-based oxide layer; and
- electrolysing dissolved alumina in the same or a different molten electrolyte using the conditioned anode structure to evolve oxygen thereon and produce aluminium on a facing cathode.

10. The method of claim 9, wherein the dense and coherent integral iron-based oxide layer formed by said polarising step of the conditioning is further formed during electrolysis by slow oxidation of the metallic anode structure at the metallic structure/oxide layer interface, optionally. constituents of the dense and coherent integral iron-based oxide layer slowly dissolve into the electrolyte during electrolysis, preferably at a rate corresponding to the oxidation rate of the metallic anode structure.

11. The method of claim 10, comprising maintaining in the aluminium-production molten electrolyte an amount of dissolved iron species and dissolved alumina sufficient to inhibit significantly dissolution of constituents of the dense and coherent integral iron-based oxide layer.

12. The method of any one of claims 9 to 11, comprising maintaining the aluminium-production molten electrolyte at a temperature below 960°C, preferably between 840°C and 940°C.

13. The method of any one of claims 9 to 12, wherein the aluminium production molten electrolyte contains NaF and AlF₃ in a molar ratio in the range from 1.2 to 2.4.

14. The method of any one of claims 9 to 13, wherein the concentration of alumina dissolved in the aluminium production molten electrolyte is below 10 weight%, preferably between 5 weight% and 8 weight%.

15. The method of any one of claims 9 to 14, wherein alumina-depleted electrolyte is circulated away from the electrochemically active iron-based oxide layer, enriched with alumina, and alumina-enriched electrolyte is circulated towards the electrochemically active iron-based oxide layer.

16. An aluminium electrowinning anode structure comprising an iron-based alloy metallic outer part with an active anode surface which is essentially metallic and free of any ceramic compounds of metals from the metallic anode structure and which is covered with a temporary protection medium that substantially prevents ceramic-forming reactions at the essentially metallic anode surface, which medium is separable from the active surface prior to or upon immersion into the molten electrolyte.

17. The anode structure of claim 16, wherein the temporary protection medium is removable prior to immersion into the electrolyte and/or soluble in the electrolyte.

18. The anode structure of any one of claims 16 to 17, wherein the temporary protection medium comprises one or more solid layers.

19. The anode structure of claim 18, wherein at least one solid layer comprises a ceramic, such as alumina, and/or at least one solid layer comprises a metal, in particular a reactable metal, such as aluminium, iron, copper, chromium or yttrium, for reacting with possibly diffusing reactive gases.

20. The anode structure of claims 18 or 19, wherein at least one solid layer comprises a polymer, the anode structure being optionally wrapped under vacuum or inert gas in the solid polymer layer.

21. The anode structure of any one or claims 16 to 20, wherein the temporary protection medium comprises: an inert liquid, such as oil or grease; and/or an inert gas, such as nitrogen and/or carbon dioxide.

22. An aluminium electrowinning cell comprising at least one oxygen-evolving anode structure according to claim 16 and optionally. an aluminium-wettable cathode, such as a drained cathode.

## Patentansprüche

1. Verfahren zum Konditionieren einer metallischen Anodenstruktur für die Herstellung von Aluminium in einem gelöstes Aluminiumoxid enthaltenden geschmolzenen Elektrolyten, wobei die metallische Anodenstruktur anfangs einen äußeren Teil aus einer auf Eisen basierenden Legierung mit einer aktiven Anodenoberfläche aufweist, die im Wesentlichen metallisch und frei von irgendwelchen keramischen Verbindungen, insbesondere Oxiden und Fluoriden, von Metallen aus der metallischen Anodenstruktur ist, bei dem:
a) die im Wesentlichen metallische aktive Oberfläche, die frei von den keramischen Verbindungen ist, mit einer temporären Schutzschicht bedeckt wird, die für irgendwelche Spezies, die mit der aktiven Oberfläche reaktionsfähig sind, im Wesentlichen undurchlässig ist, um die aktive Oberfläche im Wesentlichen vor einem Reagieren mit irgendeiner reaktionsfähigen Spezies zu schützen, insbesondere Sauerstoff- und Fluorspezies, bis das Eintauschen in einen Sauerstoffionen enthaltenden geschmolzenen Elektrolyten erfolgt,
b) Eintauchen der metallischen Anodenstruktur mit ihrer im Wesentlichen metallischen aktiven Oberfläche, die frei von den keramischen Verbindungen ist, in den geschmolzenen Elektrolyten, wobei die temporäre Schutzschicht vor dem Eintauschen in den geschmolzenen Elektrolyten oder durch Kontakt mit dem geschmolzenen Elektrolyten entfernt wird, und
c) die eingetauchte metallische Anodenstruktur polarisiert wird, um darauf eine dichte und kohärente, integrale, auf Eisen basierende Oxidschicht zu bilden, die elektrochemisch hinsichtlich der Oxidation von Sauerstoff aktiv ist und die Diffusion von Sauerstoff in Richtung der metallischen Anodenstruktur hemmt.

2. Verfahren nach Anspruch 1, bei dem die metallische Anodenstruktur vor dem Eintauchen vorab erhitzt wird, wobei ihre im Wesentlichen metallische aktive Oberfläche frei von den keramischen Verbindungen gehalten wird, und die Schutzschicht vorzugsweise wärmestabil ist.

3. Verfahren nach Anspruch 1 oder 2, bei dem die metallische Anodenstruktur vor dem Eintauchen vorab in einer Atmosphäre vorab erhitzt wird, die im Wesentlichen frei von irgendwelchen Spezies ist, die mit der aktiven Oberfläche reaktionsfähig sind.

4. Verfahren nach einem der vorhergehenden Ansprüche, bei dem der äußere Teil aus der auf Eisen basierenden Legierung Nickel und/oder Kobalt umfasst.

5. Verfahren nach einem der vorhergehenden Ansprüche, bei dem der äußere Teil aus der auf Eisen basierenden Legierung ein oder mehrere Elemente ausgewählt aus Kupfer, Molybdän, Mangan, Titan, Tantal, Wolfram, Hafnium, Vanadium, Zirkonium, Niob, Chrom, Kobalt, Aluminium, Silicium, Kohlenstoff und den seltenen Erdmetallen, insbesondere Yttrium umfasst.

6. Verfahren nach Anspruch 4, bei dem der äußeren Teil aus auf Eisen basierender Legierung im Wesentlichen aus:
- 45 bis 55 Gew.-% Eisen,
- 15 bis 55 Gew.-% insgesamt an Nickel und/oder Kobalt,
- 0 bis 30 Gew.-% Kupfer und
- 0 bis 10 Gew.-% insgesamt an einem oder mehreren weiteren Elementen
besteht.

7. Verfahren nach einem der vorhergehenden Ansprüche, bei dem die metallische Anodenstruktur eine Gießlegierung ist, wobei die Struktur gegebenenfalls vor dem Eintauchen in den geschmolzenen Elektrolyten abgeschreckt wird und/oder vor dem Eintauchen in den geschmolzenen Elektrolyten einer Glühbehandlung unterzogen wird.

8. Verfahren zum Konditionieren oder Rekonditionieren einer metallischen Anodenstruktur für die Herstellung von Aluminium in einem gelöstes Aluminiumoxid enthaltenden geschmolzenen Elektrolyten, wobei die metallische Anodenstruktur einen äußeren Teil aus einer auf Eisen basierenden Legierung mit einer Oberfläche umfasst, die mit keramischen Verbindungen, insbesondere Oxiden und Fluoriden, von Metallen aus dem äußeren Teil bedeckt ist, bei dem
- im Wesentlichen alle keramischen Verbindungen von der Oberfläche des äußeren Teils entfernt werden, um eine im Wesentlichen metallische aktive Anodenoberfläche zu bilden, und dann
- die metallische Anodenstruktur mit ihrer im Wesentlichen metallischen aktiven Anodenoberfläche, die frei von irgendwelchen keramischen Verbindungen ist, gemäß einem der vorhergehenden Ansprüche konditioniert wird.

9. Verfahren zum elektrolytischen Gewinnen von Aluminium, bei dem
- eine metallische Anodenstruktur gemäß einem der vorhergehenden Ansprüche konditioniert wird, was den Schritt des Polarisierens einschließt, in einem geschmolzenen Elektrolyten, um auf der Anodenstruktur eine dichte und kohärente, integrale, auf Eisen basierende Oxidschicht zu bilden, und
- in dem gleichen oder einem anderen geschmolzenen Elektrolyten gelöstes Aluminiumoxid unter Verwendung der konditionierten Anodenstruktur elektrolysiert wird, um daran Sauerstoff zu entwickeln und an der gegenüberliegenden Kathode Aluminium herzustellen.

10. Verfahren nach Anspruch 9, bei dem die dichte und kohärente, integrale, auf Eisen basierende Oxidschicht, die durch den Polarisierungsschritt des Konditionierens gebildet worden ist, ferner während der Elektrolyse durch langsame Oxidation der metallischen Anodenstruktur an der metallische Struktur/Oxidschicht-Grenzfläche gebildet wird, wobei gegebenenfalls Bestandteile der dichten und kohärenten, integralen, auf Eisen basierenden Oxidschicht sich langsam während der Elektrolyse in den Elektrolyten auflösen, vorzugsweise mit einer Rate, die der Oxidationsrate der metallischen Anodenstruktur entspricht.

11. Verfahren nach Anspruch 10, bei dem in dem geschmolzenen Elektrolyten der Aluminiumproduktion eine Menge an gelösten Eisenspezies und gelöstem Aluminiumoxid aufrechterhalten wird, die ausreicht, um eine signifikante Auflösung von Bestandteilen der dichten und kohärenten, integralen, auf Eisen basierenden Oxidschicht zu hemmen.

12. Verfahren nach einem der Ansprüche 9 bis 11, bei dem der geschmolzene Elektrolyt für die Aluminiumproduktion bei einer Temperatur unter 960 °C, vorzugsweise zwischen 840 °C und 940 °C gehalten wird.

13. Verfahren nach einem der Ansprüche 9 bis 12, bei dem der geschmolzene Elektrolyt für die Aluminiumproduktion NaF und AlF₃ in einem Molverhältnis im Bereich von 1,2 bis 2,4 enthält.

14. Verfahren nach einem der Ansprüche 9 bis 13, bei dem die Konzentration von Aluminiumoxid, das in dem geschmolzenen Elektrolyten für die Aluminiumproduktion gelöst ist, unter 10 Gew.-%, vorzugsweise zwischen 5 Gew.-5 und 8 Gew.-% liegt.

15. Verfahren nach einem der Ansprüche 9 bis 14, bei dem der an Aluminiumoxid verarmte Elektrolyt von der elektrochemisch aktiven, auf Eisen basierenden Oxidschicht wegzirkuliert wird, mit Aluminiumoxid angereichert wird, und der mit Aluminiumoxid angereicherte Elektrolyt zu der elektrochemisch aktiven, auf Eisen basierenden Oxidschicht hinzirkuliert wird.

16. Anodenstruktur für die elektrolytische Gewinnung von Aluminium, die einen metallischen äußeren Teil aus einer auf Eisen basierenden Legierung mit einer aktiven Anodenoberfläche umfasst, die im Wesentlichen metallisch und frei von irgendwelchen keramischen Verbindungen von Metallen aus der metallischen Anodenstruktur ist und mit einem Medium für einen temporären Schutz bedeckt ist, das keramisches Material bildende Reaktionen an der im wesentlichen metallischen Anodenoberfläche im Wesentlichen verhindert, wobei das Medium von der aktiven Oberfläche vor oder beim Eintauchen in den geschmolzenen Elektrolyten abtrennbar ist.

17. Anodenstruktur nach Anspruch 16, bei der das Medium für den temporären Schutz vor dem Eintauchen in den Elektrolyten entfernbar ist und/oder in dem Elektrolyten löslich ist.

18. Anodenstruktur nach einem der Ansprüche 16 bis 17, bei dem das Medium für den temporären Schutz eine oder mehrere feste Schichten umfasst.

19. Anodenstruktur nach Anspruch 18, bei der mindestens eine feste Schicht ein keramisches Material wie beispielsweise Aluminiumoxid umfasst und/oder mindestens eine feste Schicht ein Metall, insbesondere ein reaktionsfähiges Metall, wie beispielsweise Aluminium, Eisen, Kupfer, Chrom oder Yttrium umfasst, um mit möglicherweise diffundierenden reaktiven Gasen zu reagieren.

20. Anodenstruktur nach Anspruch 18 oder 19, bei der mindestens eine feste Schicht ein Polymer umfasst und gegebenenfalls unter Vakuum oder Inertgas in die feste Polymerschicht eingewickelt worden ist.

21. Anodenstruktur nach einem der Ansprüche 16 bis 20, bei dem das Medium für den temporären Schutz eine inerte Flüssigkeit wie beispielsweise Öl oder Schmiere umfasst, und/oder ein Inertgas wie beispielsweise Stickstoff und/oder Kohlendioxid umfasst.

22. Zelle zum elektrolytischen Gewinnen von Aluminium, die mindestens eine Sauerstoff entwickelnde Anodenstruktur gemäß Anspruch 16 und gegebenenfalls eine mit Aluminium benetzbare Kathode wie beispielsweise eine drainierte Kathode umfasst.

## Revendications

1. Procédé de conditionnement d'une structure anodique métallique pour produire de l'aluminium dans un électrolyte fondu contenant de l'alumine dissoute, la structure anodique métallique ayant initialement une partie externe en alliage à base fer avec une surface anodique active qui est essentiellement métallique et dépourvue de quelconques composés céramiques, en particulier des oxydes et fluorures, de métaux provenant de la structure anodique métallique, le procédé comprenant les étapes de :
a) recouvrir la surface active essentiellement métallique dépourvue dudit composé céramique avec une couche protectrice temporaire qui est sensiblement imperméable à une quelconque espèce pouvant réagir avec la surface active pour empêcher sensiblement la surface active de réagir avec une quelconque espèce pouvant réagir, en particulier des espèces oxygène et fluor, jusqu'à l'immersion dans un électrolyte fondu contenant des ions oxygène ;
b) immerger dans l'électrolyte fondu la structure anodique métallique avec sa surface active essentiellement métallique dépourvue desdits composés céramiques, la couche protectrice temporaire étant éliminée avant l'immersion dans l'électrolyte fondu ou par contact avec l'électrolyte fondu ;
c) polariser la structure anodique métallique immergée pour former sur celle-ci une couche d'oxyde à base de fer intégrante, dense et cohérente, qui est électrochimiquement active pour l'oxydation de l'oxygène et qui empêche la diffusion de l'oxygène vers la structure anodique métallique.

2. Procédé de la revendication 1, dans lequel, avant l'immersion, la structure anodique métallique est préchauffée avec sa surface active essentiellement métallique maintenue dépourvue desdits composés céramiques, la couche protectrice étant de préférence stable à la chaleur.

3. Procédé de la revendication 1 et 2, dans lequel, avant l'immersion, la structure anodique métallique est préchauffée dans une atmosphère qui est sensiblement dépourvue d'une quelconque espèce pouvant réagir avec la surface active.

4. Procédé d'une quelconque revendication précédente, dans lequel la partie externe en alliage à base de fer comprend du nickel et/ou du cobalt.

5. Procédé d'une quelconque revendication précédente, dans lequel la partie externe en alliage à base de fer comprend un ou plusieurs éléments choisis parmi le cuivre, le molybdène, le manganèse, le titane, le tantale, le tungstène, l'hafnium, le vanadium, le zirconium, le niobium, le chrome, le cobalt, l'aluminium, le silicium, le carbone et les métaux des terres rares, en particulier l'yttrium.

6. Procédé de la revendication 4, dans lequel la partie externe en alliage à base de fer se compose essentiellement de :
- 45-55% en poids de fer ;
- 15-55 % en poids du total de nickel et/ou de cobalt ;
- 0-30% en poids de cuivre ; et
- 0-10% en poids du total d'un ou de plusieurs autres éléments.

7. Procédé d'une quelconque revendication précédente, dans lequel la structure anodique métallique est un alliage coulé, la structure étant éventuellement trempée avant l'immersion dans l'électrolyte fondu et/ou soumise à un traitement thermique de recuit avant l'immersion dans l'électrolyte fondu.

8. Procédé de conditionnement ou de reconditionnement d'une structure anodique métallique pour produire de l'aluminium dans un électrolyte fondu contenant de l'alumine dissoute, la structure anodique métallique comprenant une partie externe en alliage à base de fer ayant une surface qui est recouverte de composés céramiques, en particulier des oxydes et des fluorures, de métaux provenant de la partie externe, ledit procédé comprenant les étapes de :
- éliminer sensiblement tous les composés céramiques de la surface de la partie externe pour former une surface anodique active essentiellement métallique ; et ensuite
- conditionner selon une quelconque revendication précédente la structure anodique métallique avec sa surface anodique active essentiellement métallique dépourvue de quelconques composés céramiques.

9. Procédé d'extraction électrolytique d'aluminium comprenant les étapes de :
- conditionner selon une quelconque revendication précédente une structure anodique métallique incluant l'étape de polarisation dans un électrolyte fondu pour former sur la structure anodique une couche d'oxyde à base de fer intégrante, dense et cohérente ; et
- électrolyser l'alumine dissoute dans le même électrolyte fondu ou un électrolyte fondu différent en utilisant la structure anodique conditionnée pour dégager de l'oxygène sur celle-ci et produire de l'aluminium sur une cathode en vis-à-vis.

10. Procédé de la revendication 9, dans lequel la couche d'oxyde à base de fer intégrante, dense et cohérente formée par ladite étape de polarisation du conditionnement est de plus formée pendant l'électrolyse par oxydation lente de la structure anodique métallique au niveau de l'interface structure métallique/couche d'oxyde, éventuellement des constituants de la couche d'oxyde à base de fer intégrante, dense et cohérente se dissolvent lentement dans l'électrolyte pendant l'électrolyse, de préférence à une vitesse correspondant à la vitesse d'oxydation de la structure anodique métallique.

11. Procédé de la revendication 10, consistant à maintenir dans l'électrolyte fondu de production d'aluminium une quantité suffisante d'espèces de fer dissoutes et d'alumine dissoute pour empêcher la dissolution de façon significative de constituants de la couche d'oxyde à base de fer intégrante, dense et cohérente.

12. Procédé de l'une quelconque des revendications 9 à 11, consistant à maintenir l'électrolyte fondu de production d'aluminium à une température en dessous de 960°C, de préférence entre 840°C et 940°C.

13. Procédé de l'une quelconque des revendications 9 à 12, dans lequel l'électrolyte fondu de production d'aluminium contient NaF et AlF₃ dans un rapport molaire se trouvant dans la plage de 1,2 à 2,4.

14. Procédé d'une quelconque des revendications 9 à 13, dans lequel la concentration d'alumine dissoute dans l'électrolyte fondu de production d'aluminium est en dessous de 10% en poids, de préférence entre 5% en poids et 8% en poids.

15. Procédé d'une quelconque des revendications 9 à 14, dans lequel l'électrolyte appauvri en alumine est mis en circulation au loin de la couche d'oxyde à base de fer électrochimiquement active, est enrichi en alumine, et l'électrolyte enrichi en alumine circule vers la couche d'oxyde à base de fer électrochimiquement active.

16. Structure anodique d'extraction électrolytique d'aluminium, comprenant une partie externe métallique en alliage à base de fer avec une surface anodique active qui est essentiellement métallique et dépourvue de composés céramiques de métaux provenant de la structure anodique métallique et qui est recouverte d'un milieu de protection temporaire qui empêche sensiblement des réactions formant des céramiques au niveau de la surface anodique essentiellement métallique, lequel milieu peut être séparé de la surface active avant ou lors de l'immersion dans l'électrolyte fondu.

17. Structure anodique de la revendication 16, dans laquelle le milieu de protection temporaire peut être éliminé avant l'immersion dans l'électrolyte et/ou est soluble dans l'électrolyte.

18. Structure anodique d'une quelconque des revendications 16 à 17, dans laquelle le milieu de protection temporaire comprend une ou plusieurs couches solides.

19. Structure anodique de la revendication 18, dans laquelle au moins une couche solide comprend une céramique, telle que l'alumine, et/ou au moins une couche solide comprend un métal, en particulier un métal pouvant réagir, tel que de l'aluminium, du fer, du cuivre, du chrome ou de l'yttrium, pour réagir avec éventuellement des gaz réactifs diffusants.

20. Structure anodique de la revendication 18 ou 19, dans laquelle au moins une couche solide comprend un polymère, la structure anodique étant éventuellement enroulée sous vide ou sous gaz inerte dans la couche polymère solide.

21. Structure anodique d'une quelconque ou des revendications 16 à 20, dans laquelle le milieu de protection temporaire comprend : un liquide inerte, tel que de l'huile ou de la graisse ; et/ou un gaz inerte, tel que de l'azote et/ou du dioxyde de carbone.

22. Cellule d'extraction électrolytique d'aluminium comprenant au moins une structure anodique à dégagement d'oxygène selon la revendication 16 et éventuellement une cathode mouillable par l'aluminium, telle qu'une cathode drainée.
